

Sept. 29, 1942.

F. BIEDERMANN

2,297,385

METHOD OF PRODUCING COMPOUND CAST BEARINGS

Filed Feb. 3, 1940



Fig. 1.



Fig. 2.

Fig. 3.



Fig. 5.



Fig. 4.



## UNITED STATES PATENT OFFICE

2,297,385

## METHOD OF PRODUCING COMPOUND CAST BEARINGS

Felix Biedermann, Berlin-Weissensee, Germany;  
vested in the Alien Property CustodianApplication February 3, 1940, Serial No. 317,207  
In Germany February 3, 1939

3 Claims. (Cl. 29—149.5)

The present invention relates to a method of producing compound cast bearings.

For the manufacture of compound cast bearings, in particular for the production of such bearings on a large scale, methods are known according to which during casting of the friction bearing metal the supporting portion has not the cylindrical form corresponding to that of the bearing portions. Steel bands or steel plates are used which are bent after applying the bearing metal and after a corresponding division into individual bearing boxes. In this manner a nearly continuous production of compound cast bearings is obtained which saves time and individual work and therefore renders cheap the manufacture of such bearings. The forming by the bending operation replaces the otherwise required expensive finish of the steel blank to be lined which is characterized by a large consumption of material and a large removal of metal by cutting. Such methods, however, are rather complicated and in particular are not adapted to be used, if bearing metal alloys, for instance lead bronzes, are to be treated which from the standpoint of casting technique offer great difficulties, because the steel and the alloy may be welded together under certain condition only, whereas harmful segregations cannot be prevented. Moreover, in this manner at the best half bearing boxes only may be produced.

Methods for the manufacture of bearings by internally lining cylindrical tubes are known according to which a tube provided at the upper end with supply means for suction or compressed air is lowered into the melt, whereupon the melt, i. e. first of all borax and then bronze, are drawn in by vacuum. The excess metal is then pressed out again, whereby eventually a core may be introduced. The compound cast bodies produced in this manner are then eventually by dividing further treated to obtain a plurality of bearing boxes. For a production on a large scale this method, however, is not very well adapted, because it is rather complicated and requires a complicated device.

The present invention relates to a method by means of which compound cast bearings of best properties may in a simple manner cheaply be produced which are free of the above mentioned drawbacks.

To obtain the object aimed at according to the invention, a special blank is used which is of exactly or nearly exactly the desired shape, for instance cylindrical, of the supporting portion. The blank, moreover, is from the beginning

5 formed as a vessel of one piece. In this manner the known lining of compound cast bearings in an upright mold may be carried out without using a special mold or any other additional device which affects the cooling. In particular casting is effected without the use of a sand grain or the like as lower closure. The blank in this manner may very simply be treated in a manner known per se with a fluxing agent.

Other objects and advantages of the invention will be apparent during the course of the following description. In the accompanying drawing, forming a part of this specification, and in which like numerals are employed to designate like parts throughout the same,

Figure 1 is a sectional view of several steel blanks arranged to receive molten bearing metal in accordance with the invention,

Figure 2 is a sectional view of a blank having a mandrel inserted therein to force out the excess bearing metal,

Figure 3 is a sectional view of the steel blank lined with the bearing metal at the completion of the operation shown in Figure 2,

Figure 4 is a sectional view of the bearing with the bottom severed to form a bearing ring, and,

Figure 5 is a perspective view of the bearing severed in half to form a pair of half-bearing boxes.

30 A larger number of the vessel-like cylindrical steel blanks are successively lined with bearing metal 2 by being filled with the melt 3 from above, while standing in a vertical position. After heating up of the steel blank, the superfluous molten material is pressed out for instance by introducing a mandrel 4, as seen in Figure 2 and the steel blank obtained in this manner is chilled in water as quickly as possible. The superfluous bearing metal, however, may also be removed in a suitable manner after cooling.

40 Then for the production of a bearing ring as seen in Figure 4 the bottom 5 is severed. For the production of half bearing boxes the blank is once more subdivided as seen in Figure 5, so that by a corresponding forming two halves A and B of the desired radius are directly obtained.

45 A blank according to the invention for the supporting box may be produced in the usual manner. According to one modification of the invention chiplessly deformed, particularly drawn bodies, are used. The operation may be started by using a sheet metal of nearly the thickness of the wall of the bearing portion desired later on, allowing the most simple manufacture of the body on a large scale.

An essential advantage of the present invention consists in avoiding any substantial deformation of the cast blank in spite of the production on a large scale. The deformation of compound cast plates to bearing portions must, as is quite evident, have a harmful effect upon the quality of the finished bearing portion, as hereby the structure as well as the connection of the lined bearing material is affected.

It is to be understood that the form of the invention, herewith shown and described, is to be taken as a preferred example of the same, and that various changes in the shape, size and arrangement of parts may be resorted to without departing from the spirit of the invention, or the scope of the subjoined claims.

What I claim is:

1. In a method of the character described, placing a cup-shaped metal blank in an upright position, pouring fusible bearing metal in molten condition into the blank through the open top thereof, subsequently ejecting some of said bearing metal while in molten condition from the blank while leaving a sufficient quantity thereof within the blank to line the latter, and then after 15 the lining is bonded to the blank and cool, severing the bottom of the blank and the portion of the bearing blank which lines the bottom of the blank and thus producing a bearing ring.

2. In a method of the character described, placing a cup-shaped metal blank in an upright position, filling said blank with fusible bearing metal in molten condition, subsequently heating the blank and the bearing metal contained therein, ejecting all of the bearing metal from the blank with the exception of a portion thereof forming a lining for the blank, then after the fusible metal is bonded to the blank and cool, removing the bottom of the blank and the portion of the bearing metal which lies said bottom and thus producing a bearing ring.

3. In a method of the character described, placing a cup-shaped steel blank in an upright position, filling said blank with fusible bearing metal in molten condition, subsequently heating the blank and the bearing metal contained therein, ejecting all of the bearing metal from the blank with the exception of a portion thereof forming a lining for the blank, then after the fusible metal is bonded to the blank and cool, removing the bottom of the blank and the portion of the bearing metal which lines said bottom and thus producing a bearing ring, and finally cutting the bearing ring lengthwise thereof and thereby forming half bearing boxes.

FELIX BIEDERMANN.